

## UNITED STATES PATENT OFFICE

WILLIS A. BOUGHTON, OF CAMBRIDGE, MASSACHUSETTS, ASSIGNOR TO BENNETT BOX COMPANY, OF BOSTON, MASSACHUSETTS, A CORPORATION OF MASSACHUSETTS

## PLASTIC PROCESS

No Drawing.

Application filed January 7, 1925. Serial No. 1,037.

This invention relates to improvements in plastic processes. More particularly it relates to processes for dealing with sheets of stiffening material suitable for use for toe boxes for shoes, although it is applicable for dealing with other materials which it may be desired to transmute between a firm state and a plastic or workable state.

In the ordinary commercial processes of making toe boxes it is customary to soften the material, for the lasting operation, by the addition of heat or by dipping the material into a solvent. There are objections to both of these processes. When heat is used, the softening must be executed always at least twice, just before slipping into the toe for "pulling over" and again when the toe is lasted or "wiped in" to produce an even smooth toe. When a solvent is used some loss of stiffening material results by the process of solution; and in the case of the materials of this sort most commonly used, celluloid or cellulose esters, great speed in handling the softened box is required in order to get it lasted before the very volatile solvent evaporates; the wastage of the solvent is extensive; and the fire hazard is often an important consideration.

It is a feature of the present invention that it provides a means for softening without either heating or dissolving the stiffening material. Although the invention has been developed in connection with toe boxes for shoes, the improved stiffening material disclosed herein and the methods for dealing with stiff materials may be used for other purposes so far as they are suitable.

The invention is illustrated as it may be applied to stiffening materials, usually organic, such as pitch or rosin which are ordinarily softened by heat, or such as celluloid or any cellulose ester which are ordinarily softened by a solvent liquid. The softening is effected by the action of a volatile liquid, upon whose evaporation the stiff condition recurs; and the evaporation may be arranged to occur sufficiently slowly and under suitable conditions to favor the recovery of the liquid.

Softeners provided by the invention work

on the following principle: To a volatile liquid in which the organic stiffener is soluble, or to a mixture of liquids if preferred, is added another volatile liquid or mixture which is soluble or miscible in the first in all proportions, but in which the organic stiffener is insoluble. This mixture may be a vehicle, as it were, for other liquids of either type whose presence may be desired for various purposes, or may be controlled in its action by the addition of comparatively non-volatile liquid to alter the volatility of the resulting mixtures or to alter the solvent power, or rate of action, or for other effects. The working liquid having been prepared according to the needs of the operation in hand and results desired, the stiffener material, when immersed in it, gradually becomes soft, the softness progressing from the surface inward, until the whole is non-resiliently flexible, somewhat like a cloth wet with water. Nevertheless the stiffener does not leave the felt or other support on which it is carried and enter the liquid. That is, it does not dissolve in the ordinary sense. Even when suspended for hours in the softening liquid no stiffener is lost in solution, if the proportions of solvent to non-solvent are correct, and in the absence of high boiling or molecularly dispersing solvents of certain kinds. When such a softened box sheet is squeezed, some of the softened stiffener may indeed stick to the fingers, if the concentration of solvent is great enough, but when in a pile each sheet may be separated from its neighbors without undue sticking. When the softened box is removed from the working liquid and exposed to the air or to any drying medium it loses the working liquid by evaporation or other process, and when dry is found hardened to approximately original condition. This occurs with such a slow time factor that the softness continues, after removal from the liquid bath, during an ample period in which the lasting may be carried out in an efficient manner, notwithstanding the delays which occur in passing material from one operation to another in ordinary factory practice. The box thus softened lasts in the toe easily. The length of time of drying de-

pends on various specific conditions of operation, composition of softening liquid, thickness of stiffened sheet, temperature, etc. The resulting box has been found to be in every 5 way as good as those produced from similar stiffening material by the commonly practiced processes of heating and in some ways better than such. In addition it is to be observed that the process is cleanly; that the 10 material remains soft long enough to be used on shoe making processes that cannot use the heating method, such as the turn-shoe process; and that the method appears to produce a smoother toe than the old process. The absence of heat removes danger to the leather; 15 the process is cheaper to operate than those using heat; and the box itself cheaper to make. And it is not necessary to use a highly inflammable liquid.

20 An illustrative example of the practice of the invention follows: A sheet of suitable supporting material is first saturated with an organic stiffener of any desired or suitable sort, which may for example comprise melted 25 rosin, or a mixture of gums, or celluloid or any cellulose ester. The supporting means may consist of loosely matted cellulose such as paper stock, kraft or sulfite pulp, re-pulped newspaper stock, or felt or cloth; and in case 30 the stiffening material be such as not to need these supporting sheets, as in the case of some celluloid stiffeners, the supporting sheet may be omitted. The prepared sheet is then cut with a die into the suitable form for the 35 toe box, known sometimes as a "disc," and may be skived. For the purposes of the present illustrative example it may be assumed that the stiffener is made of rosin, with dye if desired. Using a supporting sheet of re- 40 pulped material 70 mils thick preferably including a thin cloth reinforcement or support, and saturated with rosin applied in molten form, the excess of stiffener liquid may be squeezed out by rolling between 45 heated rollers. Then if desired the pulp may be further compressed to 50 mils by rerolling the cold saturated sheets between hot rolls. This molten composition thus having been 50 impregnated into a suitable supporting sheet, and cooled to solid and stiff form, the prepared sheet can be shipped to market or otherwise may await its use in the shoe. When they are to be used, such sheets can be 55 died to shape; can be skived satisfactorily; and may then be immersed in a softening liquid which in the present example may contain approximately 30 to 35 parts by volume of denatured alcohol No. 1 (a mixture of 90% ethyl alcohol and 10% methanol) mixed 60 with 70 to 65 parts of water. The stiff sheet may become soft enough to last in the toe of a shoe within half an hour to five hours, depending on several controllable variables such as temperature, thickness of sheet, etc.

65 The lasting is easily performed. The oper-

ator does not need to hurry his work, the operation is clean and not smeary, and the quality of the leather is not in danger of being injured. The last may be withdrawn after three hours; and the toe is hard enough 70 to be worn after one to three days. The drying may be accomplished in an enclosure so that the solvent liquid is recovered to be used over and over again. The approximate proportion of the constituents must however be maintained, by occasional observation and addition of fresh material as may be needed from time to time, especially if careful effort 75 is not made to recover the solvent liquid as fully as possible.

If some tackiness of the box is desired, in order that it may adhere to the doubler, leather or lining of the shoe, this can easily be secured by using a greater concentration or proportion of the dissolving component of the mixed liquid. Should a softer box be required, this may be produced by adding to the softening liquid a portion of comparatively non-volatile solvent for the stiffener. One half per cent of such a liquid as xylene 90 or toluene will produce a toe which is notably more flexible. Such a toe holds the shape of the last, but because it tends to soften under the heat of the foot, it will easily conform to the shape of the foot, which is an 95 advantage that may be desired by some as it markedly decreases the discomfort which is ordinarily attendant upon the "breaking in" of new shoes.

By incorporation of gum of various qualities and proportions in the stiffener the characteristic of the stiffened material may be considerably altered. In particular a composition can be chosen whose melting or softening point, under heat, is safely higher than that of the composition at present commonly used in those processes in which the softening for lasting is effected by heating, in which the softening temperature is often so low that in the finished shoe the toe loses its shape if the wearer accidentally rests it close to a steam pipe. Should a permanently softer material be desired it can be obtained by substituting in part a non-drying oil, such as castor oil or cotton seed oil, or a drying oil such as linseed or tung oil, or by some combination of constituents of a gummy or waxy nature.

This process is also well adapted to the softening of sheets of cloth, felt, etc. used for other purposes, stiffened with the said types of stiffening material, and is not necessarily confined either to shoe boxes or to materials using pulp.

I am unable to explain at the present time 125 the exact nature of the physico-chemical process by which this type of mixed liquid acts as a softener and not as a solvent, but it seems possible (on the principle that if liquid A is soluble in liquid B, then liquid B must be 130

- soluble to some extent in liquid A) that when the stiffener is placed in contact with the mixed liquid it acts as a solvent for that constituent or for those constituents which are selected as solvents for the stiffener, drawing into itself enough of this solvent to form a semi-fluid mixture, until it reaches an equilibrium in which the non-solvent has as much attraction for this solvent liquid as the stiffener has. At that point no more enters, or at least as much leaves as enters; and the presence in the mixed liquid of a constituent in which the stiffener is insoluble prevents any (or at least prevents all except a very little) of the stiffener from passing into the liquid. It is evident that the softening of the stiffener or other solid results from some degree of absorption of the solvent into its own mass because with use the liquid becomes weaker in the solvent and its strength can be restored by adding more of the solvent. And the going of the stiffener into solution in the liquid is negated by the absence of discoloration of the liquid.
- The purpose of having the liquid volatile is to make the operation complete within a commercially desirable period of time. The volatile liquid that dissolves the stiffener may be any suitable solvent, therefore, such as alcohol, acetone, or any mixture of these, or other solvent. The non-dissolving volatile liquid or mixture of liquids, which acts as a restrainer, is one in which the stiffener is insoluble but which mixes with the first liquid, and preferably one which mixes in all proportions with it. For a rosin or celluloid stiffener, water is a useful example of a suitable restraining liquid. In the illustration above given a practical test for telling the proper proportions is to observe whether the liquid becomes discolored, which indicates that the rosin is passing into solution, and calls for a larger proportion of the restraining liquid in making the stiffener soft, if it be desired that it should not become tacky or sticky or be wasted.
- If tackiness be desired, another method is to dip the softened box into purer solvent just prior to lasting.
- In general, for the above stiffener, one may employ a mixture of ethyl and/or methyl alcohol and water in any of various proportions, depending on the nature of the stiffener and the speed and degree of softening and of evaporation desired. To these liquids may be added any other desired substance that will dissolve therein in order to add any specific properties. Thus, with such a softening liquid may be mixed other solvents of the stiffener as ketones, hydrocarbons, ethers, etc., each of which may add its peculiar effect to the mixture. Xylene and other coal tar solvents, for example produce a tackiness as well as a softening. It is also to be observed that by the addition of solids (either inorganic salts or organic material) which go into solution, the solution may produce other specific desirable effects, among which may be a dyeing of the stiffener.
- For a stiffener of different type the softening mixture must be selected differently in accordance with the principles stated. Thus, where the stiffener is a gelatin or glue, the softening liquid may have water as its dissolving agent and a suitable inorganic liquid in which the glue does not dissolve, but which mixes with or dissolves in the water, as the restraining agent. To this may be added formaldehyde to toughen the glue and render it resistant to water. Potassium bichromate also will tend to render the glue insoluble in water after being lasted in the shoe.
- For a specific example of softening a stiffened sheet of the type last mentioned, a piece of glue-coated buckram may be immersed in a mixture of 25 parts of water which is the solvent liquid and 75 parts of acetone which is the non-solvent liquid. In one such instance this was found to soften within an hour and a half to a flexibility like that of wet sail canvas, that is to limpness; and the glue did not dissolve off upon continued soaking in the same liquid for twenty-four hours; and upon the removal and drying of the coated buckram thereafter it again became hard and stiff.
- In the practice of the invention it appears that the fibers of the supporting material such as cloth aid materially in the effect of the solvent. This is indicated by the fact that a pure rosin mixture after many hours immersion in the softening liquid described for rosin shows marked softening of the surface, but not penetration throughout, the softening extending beneath to a depth of about 0.2 to 0.3 millimeters. But where the rosin is carried on a supporting material the entrance of the liquid through the fibers aids the penetration of the solvent to interior surfaces of the stiffening material with consequent softening in the interior of the mass as well as at its surface. Rapidity of softening will be influenced by the closeness of fibers to one another and by the corresponding thinness of layer of rosin around each fiber.
- In the appended claims the single term "alcohol" is used in order to avoid the use of alternative phraseology, but it will be understood that this is not so restrictive in meaning as to exclude derivatives or other substances which are equivalents of alcohol, of which many are known.
- I claim as my invention:
1. A method of preparing stiffener blanks for use in shoes and the like, comprising the steps of impregnating a carrier sheet with melted rosin, permitting the rosin to harden to a stiff condition, and thereafter, prior to reshaping the stiffener blank in a shoe or

other article, introducing said blank into a liquid mixture consisting of 30 to 35 per cent by volume of solvent and 70 to 65 per cent of non-solvent, and capable of softening the stiffener blank without substantial dissolution during immersion of the blank in the liquid mixture for hours.

2. A method of preparing stiffener blanks for use in shoes and the like, comprising the 10 steps of impregnating a carrier sheet with stiffening material, permitting the stiffening material to harden to a stiff condition, and thereafter, prior to reshaping the stiffener blank in a shoe or other article, introducing 15 said blank into a liquid mixture consisting of 30 to 35 per cent by volume of alcohol and 70 to 65 per cent of water and capable of softening the stiffener blank without substantial dissolution during immersion of the blank in 20 the liquid mixture for hours.

Signed at Boston, Massachusetts, this sixteenth day of December, 1924.

WILLIS A. BOUGHTON.